

1

3,498,925

## SMOKE GENERATING COMPOSITIONS

Martin E. Gluckstein, Detroit, Ellis B. Rifkin, Southfield, and Harold A. Beatty, Grosse Point Farms, Mich., assignors to Ethyl Corporation, New York, N.Y., a corporation of Virginia  
No Drawing. Continuation-in-part of application Ser. No. 473,224, July 19, 1965. This application June 29, 1966, Ser. No. 561,364

The portion of the term of the patent subsequent to Sept. 3, 1985, has been disclaimed  
Int. Cl. C09k 3/30; C06d 3/00

U.S. CL. 252—305

8 Claims

### ABSTRACT OF THE DISCLOSURE

A smoke agent consisting essentially of (a) a mixture of organometallic and organometallic hydride compounds such as triethylaluminum and diethylaluminum hydride, (b) an aromatic substance having up to three carbocyclic aromatic, six-membered rings and from six to 20 carbon atoms, said aromatic substance being composed solely of carbon and hydrogen, e.g.,  $\alpha$ -methylnaphthalene, and (c) a component selected from petroleum oil and mixtures of petroleum oil and fluorocarbons. Smoke is produced by exposing the smoke agent to the atmosphere.

This application is a continuation-in-part of applicant's prior copending application Ser. No. 473,224, filed July 19, 1965, now U.S. Patent No. 3,400,082.

This invention relates to agents which produce smoke. More specifically, it relates to smoke-producing agents containing a mixture of organometallic and organometallic hydride compounds. In a highly preferred embodiment, this invention relates to smoke-producing formulations which contain a mixture of organoaluminum and organoaluminum hydride compounds.

Many of the smoke-producing formulations proposed in the past have serious deficiencies. For example, they may be too expensive. Similarly, many smokes produced by prior art smoke agents are toxic, corrosive or irritating to the skin and eyes. Thus, in many instances, personnel anticipating contact with smoke must wear protective clothing and use a breathing apparatus to obviate untoward effects produced by the smokes. Such protective measures are costly, reduce personnel efficiency and present logistic problems.

For certain operations by the armed forces, law enforcement agencies and the like, non-irritant, non-toxic and non-flammable obscuring smokes are desired. To avoid or minimize the deleterious consequences arising from the use of hazardous smokes, prior workers have proposed that smokes be generated from petroleum oils using heat sources such as specially designed heaters, turbine or diesel engines, or from oils or water in combination with certain chemical agents. In all of these instances, bulky, complex equipment is required which presents logistic problems and renders these methods impractical in certain instances; for example, in aerial and jungle operations.

Smoke-producing agents commonly employed today, e.g., FS (sulfur trioxide-chlorosulfonic acid) and FM (titanium tetrachloride), which depend upon the reaction of the moisture in the atmosphere, vary markedly in efficiency depending upon the humidity of the atmosphere at the locus of use. The smoke formulations provided by this invention do not depend solely upon a reaction with atmospheric moisture but rather, to a large extent, upon the presence of atmospheric oxygen. Hence, the agents of this invention do not vary so widely in efficiency and quantity of smoke produced as do the above named and

2

designated prior art formulations. However, the smoke-producing formulations of this invention can produce smoke by reacting with water or oxygen. This is an important feature of this invention.

In our copending parent application Ser. No. 473,224, filed Aug. 19, 1965, now U.S. Patent No. 3,400,082, we have disclosed a new type of smoke agents having properties superior to the conventional smoke agents. The smoke agents covered by our copending application consist essentially of aluminum trialkyl, and aromatic hydrocarbon and a petroleum lubricating oil. The smoke agents of the present invention, while possessing all superior properties of the agents of our copending application, also contain additional beneficial properties. For example, the smoke agents of the present invention produce smoke, as the formulations in the copending application, merely by coming in contact with oxygen and/or moisture. However, the agents of this invention are more stable than the agents in our copending application and, therefore, in some instances may be of even greater value than the compositions disclosed in our copending application.

Thus, an object of this invention is to provide improved smoke-producing agents which do not have many of the deficiencies of the prior art smoke-producing agents and/or methods. A further object is to provide non-irritant, non-toxic, and non-flammable obscuring smokes. Additional objects will be apparent from the following detailed description and appended claims.

The objects of this invention are accomplished by providing smoke-producing formulations containing a mixture of organometallic compounds.

Essentially, the smoke formulations of this invention comprise a mixture of an organometallic and organometallic hydride compounds, and one or more diluents and/or flame suppressants to control the rate of oxidation and/or hydrolysis of the organometallic compounds. In a preferred embodiment, the smoke formulations of this invention comprise an organometallic compound, an aromatic substance, petroleum oil, and/or a fluorocarbon. In a very highly preferred embodiment, this invention provides a smoke agent consisting essentially of:

(a) A mixture of an alkyl aluminum having the formula  $R_3Al$  and an alkyl aluminum hydride having the formula  $R_xAlH_y$  wherein R is an alkyl radical solely composed of carbon and hydrogen and having up to six carbon atoms, and x and y are one or two;

(b) An aromatic compound having up to three carbocyclic aromatic six-membered rings and from 6 to 20 carbon atoms, said aromatic compound being solely composed of carbon and hydrogen, and

(c) A petroleum oil.

As stated above, the smoke-producing formulations of this invention contain a mixture of organometallic compounds. Compounds of aluminum, boron and zinc are preferred. Applicable organoaluminum compounds include those having the formula

$(R_3Al)_2$  or  $R_3Al$

wherein R is an organic radical having up to six carbon atoms, said radical being selected from alkyl or aryl groups. Most preferably, R is an alkyl group having up to six carbon atoms which is solely composed of carbon and hydrogen.

Applicable organoaluminum hydrides include those having the empirical formula:

$R_xAlH_y$

wherein R is an organic radical having up to six carbon atoms, said radical being selected from alkyl and aryl groups, and x and y are one or two. Preferably, R is an alkyl group having up to six carbon atoms which is solely composed of carbon and hydrogen.

In addition to the aluminum compounds formulated above, boron compounds having the formulae:



wherein R is an alkyl or aryl group having up to six carbon atoms and x and y are one or two, can also be employed. Similarly, zinc compounds having the formulae:



wherein R has the same significance as defined above can also be used.

Highly preferred organoaluminum compounds employed in this invention include tri-n-propylaluminum, tri-n-butylaluminum, triisobutylaluminum, tri-n-amylaluminum, tri-sec-amylaluminum, tri-n-hexylaluminum, tri-phenylaluminum, ethyldiphenylaluminum, and the like, and mixtures thereof. A most highly preferred aluminum alkyl is triethylaluminum.

Highly preferred organoaluminum hydrides employed in this invention are diethylaluminum hydride, dimethylaluminum hydride, di-n-propylaluminum hydride, diisopropylaluminum hydride, diisobutylaluminum hydride, ethylmethylaluminum hydride, ethyl-n-propylaluminum hydride, isopropylisobutylaluminum hydride, and the like, and mixtures thereof.

All the organic radicals bonded to the metal atom or atoms (in the organometallic compounds employed in this invention) need not be identical. For example, two or three different radicals can be bonded to aluminum. Compounds of this type are illustrated by dimethyl ethyl aluminum, diethyl methyl aluminum, methyl diisopropyl aluminum, methyl hexyl butyl aluminum, and the like. Thus, the triorgano aluminum compounds applicable in this invention include compounds having the formula  $RR'R''Al$  wherein R, R' and R'' are alike or different alkyl radicals of one to six carbon atoms. Diorganoaluminum hydrides include compounds having the formula



wherein R and R' are alike or different alkyl radicals of one to six carbon atoms as exemplified above.

Whenever a triorganoaluminum compound is mixed with a diorganoaluminum hydride, the resulting composition does not remain merely as a physical mixture of two specific compounds. Under such conditions, molecular rearrangement or disproportionation takes place. Thus, the organic and the hydrogen radicals exchange until an equilibrium is obtained. The end result is that the composition is not merely a mixture of two compounds, but a mixture of many compounds containing compositions intermediate between the two original compounds.

The operation of disproportionation may be illustrated by the following example. If originally triethylaluminum, triisobutylaluminum and diethylaluminum hydride are mixed, the resulting disproportionation product will contain the following intermediate compounds: diethylisobutylaluminum, ethylisobutylaluminum hydride, ethyldiisobutylaluminum, and diisobutylaluminum hydride. Similar disproportionation takes place when mixtures of triorganoboron and diorganoboron hydride are employed.

In addition to the metallic compounds noted above, preferred formulations of this invention also contain an aromatic compound. Applicable aromatic materials are those which have one carbocyclic aromatic six-membered ring or from two to three fused carbocyclic aromatic six-membered rings. Preferably these compounds are solely composed of carbon and hydrogen and most preferably, they also contain from 6 to about 20 carbon atoms. Preferred substances of this type have up to 20 carbon atoms and are selected from the class consisting of alkyl-substituted benzene such as xylenes, naphthalene, alkyl-substituted naphthalenes, acenaphthene, alkyl-substituted acenaphthenes, fluorene, alkyl-substituted fluorenes, phenanthrene, alkyl-substituted phenanthrenes, anthracene, and alkyl-substituted anthracenes. Of these compounds, naph-

thalene and the alkyl-substituted naphthalenes are preferred. Highly preferred alkyl naphthalenes are  $\alpha$ -methylnaphthalene,  $\alpha$ -ethylnaphthalene, and  $\beta$ -methylnaphthalene. A very highly preferred aromatic substance is  $\alpha$ -methylnaphthalene.

The third major ingredient in the preferred formulations of this invention is a petroleum oil. In general, any petroleum oil can be employed. A preferred oil is mineral oil such as USP white mineral oil. A very highly preferred oil is Neutral No. 75 oil which is a distilled solvent-refined, dewaxed petroleum oil having a viscosity in Saybolt Universal Seconds at 100° F. within the range of from about 70 to 80. Usually oils of this type have a viscosity in Saybolt Universal Seconds within the range from 72 to 78.

Another preferred oil is Circo XXX Light Oil which is a naphthenic oil having a viscosity in Saybolt Universal Seconds at 100° F. within the range of from about 55-60. Still another preferred oil is Circosol 410 oil which is also a naphthenic oil having a viscosity in Saybolt Universal Seconds of about 100. Generally, petroleum base oils having a viscosity in Sabolt Universal Seconds in the range of from about 40 to about 200 may be employed.

In addition to the petroleum oils described above, other petroleum fractions can also be employed. For example, ordinary heating oils, diesel oil, and kerosene may be used. Similarly, crude petroleum can be employed. One or more of the above diluents can be used. For example, crude petroleum-kerosene mixtures are applicable as well as mixtures of home heating oils and kerosene.

In general, the smoke formulations of this invention contain from about 10 to about 80 parts by weight of the organometallic compounds, from about 5 to about 50 parts of an aromatic substance of the type described above and from about 10 to about 90 parts of petroleum or petroleum-derived products (all parts are by weight). The organometallic component contains from about 10 to about 60 weight percent of organometallic hydride, and preferably from about 20 to about 40 weight percent. The preferred alkylaluminum formulations of this invention contain from about 10 to about 60 parts by weight of the organoaluminum compounds, from about 5 to about 20 parts by weight of one or more aromatic substances of the type described above, and from about 40 to about 70 parts of a petroleum lubricating oil.

In addition to the above-named ingredients, the formulations of this invention may optionally contain minor amounts, say up to about 10 percent by weight, of additives to prevent freezing, reduce flame hazards, improve solubilities or compatibilities, etc. Thus, the formulations of this invention may contain fluorocarbons such as Freons, silicones, dispersants, detergents, as well as oxidizing salts such as ammonium nitrate, permanganates, chlorates, perchlorates, etc. In addition, the compositions of this invention may optionally contain metal alcoholates such as tetraisopropyl titanate (titanium tetraisopropylate), tetra-n-butyl titanate, and the like.

Ethers are a preferred type of additional ingredient which may optionally be included in the smoke-producing formulations of this invention. In general, from about 5 to about 90 parts by weight of an ether may be included in the formulations. Like the aromatic substances discussed above, the ethers seem to have a flame suppressant effect.

The preferred ethers are polyethers; in other words, they contain two or more ether oxygen atoms. Preferred polyethers are the diethers and triethers (ethers containing 2 and 3 ether oxygen atoms, respectively) having up to about 20 carbon atoms.

The diethers which are applicable herein are represented by the formula



In this formula, R is a bridging group, that is, an alkylene radical of a branched or (preferably) a straight chain

containing from one to about six carbon atoms. In addition, the bridging R group may be a cycloalkyl group, that is, it may be a saturated ring containing from 4 to 6 carbon atoms. In the above formula, R' is a terminal group which may be a saturated, straight or branched chain alkyl group containing from 1 to 20 carbon atoms. In addition, R' can also be a saturated alicyclic group, that is, it may be an alicyclic ring radical containing from 4 to 6 carbon atoms. R'', like R', is a terminal group. Hence, it is selected from the same type of radicals as R'. Preferably R' and R'' are identical radicals. Most preferably, they are alkyl radicals having from 1 to 4 carbon atoms. Illustrative but non-limiting examples of diethers which are applicable in this invention include dimethoxyethane, diethoxyethane, dibutoxyethane, and the like.

The most preferably polyethers are the triethers represented by the following formula:



In this formula, R, R' and R'' have the same significance as that in the above formula which illustrates the diethers. Illustrative but non-limiting examples of triethers which are applicable in this invention include diethyleneglycol diethylether, dipropylene glycol diethylether, dibutylene glycol dimethylether, dipropylene glycol dibutylether, dihexyleneglycol diisopropylether, dihexyleneglycol dibutylether, and the like. Very highly preferred triethers are diethyleneglycol dimethylether and diethyleneglycol dibutylether. Other polyethers such as triethyleneglycol dialkylethers can also be used.

The formulations of this invention can be prepared in any convenient manner. It is only necessary to mix the desired ingredients in the desired amounts. In many instances, it is preferable to mix the ingredients under a blanket of an inert atmosphere. Many inert gases can be employed to supply the inert atmosphere, e.g., nitrogen, neon, argon, and the like. Because of its low cost and availability, nitrogen is the preferred inert gas.

The smoke formulations of this invention produce smoke upon exposure to oxygen or moisture. Exposure to these materials is conveniently carried out by rupturing a vessel containing the formulations or by flowing the formulation through a valve and nozzle.

The following examples illustrate the smoke-producing formulations of this invention and are non-limiting. All parts are by weight unless otherwise noted.

#### EXAMPLE 1

A smoke-producing formulation was prepared by mixing the following ingredients in the amounts stated under nitrogen:

|                                                                            | Parts |
|----------------------------------------------------------------------------|-------|
| Triethylaluminum-diethylaluminum hydride (containing 28±2% of the hydride) | 25    |
| α-Methylnaphthalene                                                        | 10    |
| Circosol 410 oil                                                           | 65    |

This formulation is activated by oxygen and/or moisture in the air to produce a dense white smoke. The formulation is a clear mobile liquid at temperatures above -20° F. The above formulation is chemically stable under storage conditions of -40° F. to 120° F. The density of the material is about 0.85 gram per ml.

#### EXAMPLE 2

A smoke-producing formulation was prepared by mixing the following ingredients in the amounts stated under nitrogen:

|                                                                  | Parts |
|------------------------------------------------------------------|-------|
| Triethylaluminum-diethylaluminum hydride (containing 28±2% DEAH) | 20    |
| α-Methylnaphthalene                                              | 10    |
| Circosol 410 oil                                                 | 70    |

The properties and smoke producing ability of this formulation is substantially the same as described in Example 1.

#### EXAMPLE 3

5 A smoke-producing formulation was prepared by mixing the following ingredients in the amounts stated under nitrogen:

|                                          | Parts |
|------------------------------------------|-------|
| Triethylaluminum-diethylaluminum hydride | 30    |
| Dibromotetrafluoroethane (Freon-114 B2)  | 15    |
| Neutral No. 75 oil                       | 55    |

#### EXAMPLE 4

15 A smoke-producing formulation was prepared by mixing the following ingredients in the amounts stated under nitrogen:

|                                          | Parts |
|------------------------------------------|-------|
| Triethylaluminum-diethylaluminum hydride | 30    |
| α-Methylnaphthalene                      | 12.4  |
| Dibromotetrafluoroethane (Freon-114 B2)  | 5     |
| Neutral No. 75 oil                       | 52.6  |

#### EXAMPLE 5

25 A smoke-producing formulation was prepared by mixing the following ingredients in the amounts stated under nitrogen:

|                                          | Parts |
|------------------------------------------|-------|
| Triethylaluminum-diethylaluminum hydride | 30    |
| α-Methylnaphthalene                      | 12.4  |
| Dibromotetrafluoroethane (Freon-114 B2)  | 10    |
| Neutral No. 75 oil                       | 47.6  |

#### EXAMPLE 6

35 A smoke-producing formulation was prepared by mixing the following ingredients in the amounts stated:

|                                          | Parts |
|------------------------------------------|-------|
| Triethylaluminum-diethylaluminum hydride | 30    |
| α-Methylnaphthalene                      | 5     |
| Dibromotetrafluoroethane (Freon-114 B2)  | 12.5  |
| Neutral No. 75 oil                       | 52.5  |

45 Similar formulations are prepared by substitution of triethylaluminum-diethylaluminum hydride in Examples 1 to 6 with the following mixtures of aluminum compounds: triisopropylaluminum - diisopropylaluminum hydride, triethylaluminum - diisopropylaluminum hydride, triisopropylaluminum-diethylaluminum hydride.

#### EXAMPLE 7

55 A smoke-producing formulation was prepared by mixing the following ingredients in the amounts stated under nitrogen:

|                                          | Parts |
|------------------------------------------|-------|
| Triethylaluminum-diethylaluminum hydride | 30    |
| α-Methylnaphthalene                      | 10    |
| Dibromotetrafluoroethane (Freon-114 B2)  | 12.5  |
| Neutral No. 75 oil                       | 47.5  |

#### EXAMPLE 8

65 A smoke-producing formulation was prepared by mixing the following ingredients in the amounts stated under nitrogen:

|                                          | Parts |
|------------------------------------------|-------|
| Triethylaluminum-diethylaluminum hydride | 30    |
| α-Methylnaphthalene                      | 5.0   |
| Dibromotetrafluoroethane (Freon-114 B2)  | 12.5  |
| Circo oil                                | 52.5  |

#### EXAMPLE 9

75 A smoke-producing formulation was produced by mix-

ing the following ingredients under nitrogen in the amounts stated:

|                                          | Parts |
|------------------------------------------|-------|
| Triethylaluminum-diethylaluminum hydride | 30    |
| $\alpha$ -Methylnaphthalene              | 5     |
| Dibromotetrafluoroethane (Freon-114 B2)  | 12.5  |
| Neutral No. 75 oil                       | 26.0  |
| Circo oil                                | 26.5  |

#### EXAMPLE 10

A smoke-producing formulation is prepared by mixing the following ingredients under nitrogen in the amounts stated:

|                                          | Parts |
|------------------------------------------|-------|
| Triethylaluminum-diethylaluminum hydride | 30    |
| $\alpha$ -Methylnaphthalene              | 5     |
| Dibromotetrafluoroethane (Freon-114 B2)  | 12.5  |
| Circosol 410 oil                         | 52.5  |

In Examples 3 to 10, the content of the organoaluminum hydride is about  $28 \pm 2$  weight percent of the organo-aluminum mixture.

#### EXAMPLE 11

A smoke-producing formulation is prepared by mixing the following ingredients under nitrogen in the amounts stated:

|                                                                            | Parts |
|----------------------------------------------------------------------------|-------|
| Trimethylaluminum-isobutylaluminum hydride (containing 10% of the hydride) | 15    |
| Diethyleneglycol dimethylether                                             | 50    |
| Phenanthrene                                                               | 35    |

#### EXAMPLE 12

A smoke-producing formulation is prepared by mixing the following ingredients under nitrogen in the amounts stated:

|                                                                                       | Parts |
|---------------------------------------------------------------------------------------|-------|
| Diethylisobutylaluminum - hexylpropylaluminum hydride (containing 20% of the hydride) | 80    |
| $\alpha$ -Methylnaphthalene                                                           | 10    |
| White mineral oil                                                                     | 10    |

Similar results are obtained when anthracene, 5-n-heptylphenanthrene, 4-heptylfluorene,  $\beta$ -methylnaphthalene are employed in place of  $\alpha$ -methylnaphthalene.

#### EXAMPLE 13

A smoke-producing formulation is prepared by mixing the following ingredients under nitrogen in the amounts stated:

|                                                                            | Parts |
|----------------------------------------------------------------------------|-------|
| Trihexylaluminum - diethylaluminum hydride (containing 45% of the hydride) | 60    |
| $\alpha$ -Methylnaphthalene                                                | 5     |
| Dibromotetrafluoroethane (Freon-114 B2)                                    | 15    |
| Circosol 410 oil                                                           | 10    |
| Diethyleneglycol dimethylether                                             | 10    |

Similar results are obtained when in the above example, diethyleneglycol dimethylether is substituted by dipropoxybutane, dicyclohexyloxyethane, diethyleneglycol dibutylether, diethyleneglycol dipropylether, diethyleneglycol dihexylether, or dibutylene glycol dihexylether.

The smoke formulations of this invention produce a relatively innocuous smoke. The solid and liquid particles within the smoke are probably the oxides of the metals within the organometallic compounds, or hydrated metal oxides, as well as the components within the diluents and flame suppressants, e.g., Neutral No. 75 oil and  $\alpha$ -methylnaphthalene, respectively. Gaseous products which are likely to be included in the smokes produced by this invention are ethylene, butylene, butane, hydrogen, ethane, carbon dioxide. It is anticipated that the hydrocarbon diluents should be innocuous in the exposure time and concentration range time likely to be encountered. The metal oxides within the smokes, e.g., aluminum oxide, are generally considered to be relatively non-toxic.

It was stated earlier that the smoke compositions of this invention contain certain improved properties over the smoke compositions disclosed in our copending application Ser. No. 473,224. Some of the properties in which improvement is realized are flash point and fire point. The flash and fire points were determined by a standard method known as the Cleveland Open Cup Method, ASTM D92, described in "ASTM Standards on Petroleum Products and Lubricants" published by the American Society for Testing Materials, 1916 Race St., Philadelphia, Pa. Comparative results between the smoke formulation of this invention containing a mixture of triethylaluminum and diethylaluminum hydride and the smoke formulation in our copending application, mentioned above, containing triethylaluminum are given in the table below. Also reported in the table is the relative obscuring power of each smoke formulation. This test is conducted in the following manner: A standard amount of a smoke agent was atomized into an air stream in a smoke tunnel with the air flow rate kept as a constant. Smoke densities were measured with an Autotron Model P8L3/E8BC photocell-light source combination. The output from the photocell was amplified and recorded by a Mosley Autograph Model 680 strip chart recorder. This gave a time-transmission record. By plotting the time-transmission curve, the relative obscuring power of each smoke is obtained.

In the table, the abbreviations have the following meanings:

TEA-Triethylaluminum  
TEA-DEAH-Triethylaluminum-diethylaluminum  
hydride mixture  
Freon-114 B2-Dibromotetrafluoroethane

TABLE

| TEA | TEA-DEAH | $\alpha$ -Methyl-naphthalene | Weight Percent |                |           | XXX | Circo oil | Circosol 410 oil | Relative obscuring power, percent | Flash point, °F. | Fire point, °F. |
|-----|----------|------------------------------|----------------|----------------|-----------|-----|-----------|------------------|-----------------------------------|------------------|-----------------|
|     |          |                              | Freon-114 B2   | Neutral 75 Oil | Circo oil |     |           |                  |                                   |                  |                 |
| 30  | 0        | 0                            | 15.0           | 55.0           | 0         |     | 0         | 0                | Inconclusive                      | 174              | 178             |
| 0   | 30       | 0                            | 15.0           | 55.0           | 0         |     | 0         | 0                | 97                                | 288              | 291             |
| 30  | 0        | 12.4                         | 5.0            | 52.6           | 0         |     | 0         | 0                | 100                               | 111              | 111             |
| 0   | 30       | 12.4                         | 5.0            | 52.6           | 0         |     | 0         | 0                | 77                                | 111              | 119             |
| 30  | 0        | 12.4                         | 10.0           | 47.6           | 0         |     | 0         | 0                | 72                                | 135              | 143             |
| 0   | 30       | 12.4                         | 10.0           | 47.6           | 0         |     | 0         | 0                | 85                                | 178              | 181             |
| 30  | 0        | 5.0                          | 12.5           | 52.5           | 0         |     | 0         | 0                | 87                                | 187              | 190             |
| 0   | 30       | 5.0                          | 12.5           | 52.5           | 0         |     | 0         | 0                | 97                                | 277              | 291             |
| 30  | 0        | 10.0                         | 12.5           | 47.5           | 0         |     | 0         | 0                | Not tested                        | 180              | 183             |
| 0   | 30       | 10.0                         | 12.5           | 47.5           | 0         |     | 0         | 0                | 115                               | 288              | 298             |
| 30  | 0        | 5.0                          | 12.5           | 0              | 52.5      |     | 0         | 0                | 115                               | 190              | 190             |
| 0   | 30       | 5.0                          | 12.5           | 0              | 52.5      |     | 0         | 0                | 105                               | 298              | 302             |
| 30  | 0        | 5.0                          | 12.5           | 26.5           | 26.0      |     | 0         | 0                | Not tested                        | 199              | 208             |
| 0   | 30       | 5.0                          | 12.5           | 26.5           | 26.0      |     | 0         | 0                | 102                               | 273              | 295             |
| 30  | 0        | 5.0                          | 12.5           | 0              | 0         |     | 52.5      | 52.5             | Not tested                        | 176              | 180             |
| 0   | 30       | 5.0                          | 12.5           | 0              | 0         |     | 0         | 52.5             | 104                               | 277              | 277             |

From the above table it is seen that even though the relative obscuring power of the agents of this invention is generally similar to the obscuring power of the agents containing only triethylaluminum as the aluminum-containing component, the flash and fire points are very substantially improved. These properties are of great importance when dealing with smoke agents because the higher the flash and fire point, the more stable the agent is.

This invention is extended to cover smoke-producing formulations which contain hydrides such as boron hydrides. Furthermore, colored smokes may be attained by incorporating organometallic compounds, particularly of the pi-bonded type, whose metals form colored oxides.

Having fully described the novel compositions of this invention, their method of preparation, and their use, it is desired that this invention be limited only within the lawful scope of the appended claims.

We claim:

1. A smoke agent consisting essentially of:

(a) from about 10 to about 80 parts by weight of a mixture of an alkylaluminum and an alkylaluminum hydride having the following formulae respectively:



wherein R, R' and R'' are radicals solely composed of carbon and hydrogen and having up to six carbon atoms, said alkylaluminum hydride being in the amount of from 10 to about 60 weight percent of said mixture;

(b) from about 5 to about 50 parts by weight of an aromatic substance having up to 3 carbocyclic, aromatic, six-membered rings, and from 6 to 20 carbon atoms, said aromatic substance being solely composed of carbon and hydrogen; and

(c) from about 10 to about 90 parts by weight of a component selected from the class consisting of petroleum oils and a mixture of petroleum oils and fluorocarbons, said fluorocarbon being in the amount of up to 10 weight percent of said smoke agent.

2. The smoke agent of claim 1 wherein:

(a) said alkylaluminum and alkylaluminum hydride mixture is in the amount of from about 10 to about 60 parts by weight, and R, R' and R'' are alkyl radicals having up to 6 carbon atoms;

(b) said aromatic substance is in the amount of from about 5 to about 20 parts by weight, and

(c) said component is a petroleum oil in the amount of from about 40 to about 70 parts by weight.

3. The smoke agent of claim 2 wherein R, R' and R'' are ethyl.

4. The smoke agent of claim 2 wherein said aromatic substance is selected from the group consisting of xylene, naphthalene, acenaphthene, alkyl-substituted naphthalenes

and acenaphthenes, fluorene, alkyl-substituted fluorenes, phenanthrene, alkyl-substituted phenanthrenes, anthracene and alkyl-substituted anthracenes.

5. The smoke agent of claim 2 wherein said aromatic substance is  $\alpha$ -methylnaphthalene.

6. The smoke agent of claim 2 wherein:

(a) said mixture of alkylaluminum and alkylaluminum hydride is triethylaluminum-diethylaluminum hydride comprising about 25 parts by weight of the total composition, said mixture containing about 28 percent by weight of diethylaluminum hydride;

(b) said aromatic substance being an  $\alpha$ -methylnaphthalene comprising about 10 parts by weight of the total composition, and

(c) said petroleum oil being distilled, solvent refined, dewaxed petroleum oil having a viscosity in Saybolt Universal Seconds at 100° F. within the range of from about 40 to 200, and comprising about 65 parts by weight of the total composition.

7. The smoke agent of claim 2 wherein:

(a) said mixture of alkylaluminum and alkylaluminum hydride is triethylaluminum-diethylaluminum hydride comprising about 20 parts by weight of the total composition, said mixture containing about 28 percent by weight of diethylaluminum hydride;

(b) said aromatic substance being an  $\alpha$ -methylnaphthalene comprising about 10 parts by weight of the total composition, and

(c) said petroleum oil being distilled, solvent refined, dewaxed petroleum oil having a viscosity in Saybolt Universal Seconds at 100° F. within the range of from about 40 to 200 and comprising about 70 parts by weight of the total composition.

8. The smoke agent of claim 1 wherein:

(a) said mixture of an alkylaluminum and an alkylaluminum hydride is in the amount of from about 20 to about 60 parts by weight and R, R' and R'' are alkyl radicals having up to about six carbon atoms;

(b) said aromatic substance is in the amount of from about 5 to about 20 parts by weight; and

(c) said component is a mixture of petroleum oils and fluorocarbons in the amount of from about 40 to about 70 parts by weight of petroleum oil and in the amount of about 10 parts by weight of fluorocarbon, wherein said fluorocarbon is dibromotetrafluoroethane.

#### References Cited

#### UNITED STATES PATENTS

- |           |        |                   |           |
|-----------|--------|-------------------|-----------|
| 2,653,130 | 9/1953 | Eiseman           | 252—305 X |
| 3,400,082 | 9/1968 | Gluckstein et al. | 252—305   |

RICHARD D. LOVERING, Primary Examiner

UNITED STATES PATENT OFFICE  
CERTIFICATE OF CORRECTION

Patent No. 3,498,925 Dated March 3, 1970

Inventor(s) Martin E. Gluckstein, Ellis B. Rifkin, Harold A. Beatty

It is certified that error appears in the above-identified patent  
and that said Letters Patent are hereby corrected as shown below:

Column 2, line 6, for "Aug." read -- July --; Column 6,  
line 37, for "prepared" read -- produced --; Line 38, after  
"ingredients" insert -- under nitrogen --; Column 10, line 2,  
for "aikyl" read -- alkyl --.

SIGNED AND  
SEALED  
SER 1-1970

(SEAL)

Attest:

Edward M. Fletcher, Jr.

Attesting Officer

WILLIAM E. SCHUYLER, JR.  
Commissioner of Patents

UNITED STATES PATENT OFFICE  
CERTIFICATE OF CORRECTION

Patent No. 3,498,925 Dated March 3, 1970

Inventor(s) Martin E. Gluckstein, Ellis B. Rifkin, Harold A. Beatt

It is certified that error appears in the above-identified patent  
and that said Letters Patent are hereby corrected as shown below:

Column 2, line 6, for "Aug." read -- July --; Column 6,  
line 37, for "prepared" read -- produced --; Line 38, after  
"ingredients" insert -- under nitrogen --; Column 10, line 2,  
for "aikyl" read -- alkyl --.

SIGNED AND  
SEALED  
SEP 1 - 1970

(SEAL)

Attest:

Edward M. Fletcher, Jr.

Attesting Officer

WILLIAM E. SCHUYLER, JR.  
Commissioner of Patents